

July 31, 1951

R. O'HALLORAN

2,562,814

SULFONATE LUBRICATING GREASE

Filed March 5, 1949



Rosemary O'Halloran Inventor

By *Elwin M. Thomas* Attorney

## UNITED STATES PATENT OFFICE

2,562,814

## SULFONATE LUBRICATING GREASE

Rosemary O'Halloran, Elizabeth, N. J., assignor  
to Standard Oil Development Company, a cor-  
poration of Delaware

Application March 5, 1949, Serial No. 79,821

15 Claims. (Cl. 252—33.3)

1

The present invention relates to lubricating grease compositions, and particularly to lubricating greases prepared from lubricating oils which are thickened with materials other than the conventional soaps. The invention is particularly applicable to new types of lubricating greases which contain a mixture or a complex of oil soluble and oil insoluble materials, such as oil soluble sulfonates and oil insoluble salts of low molecular weight as the thickening agent.

Recently, several suggestions have been made that the soap content of normal lubricating greases may be largely or entirely replaced by a mixture or a complex of an oil soluble petroleum sulfonate with an oil insoluble, or relatively insoluble salt of low molecular weight acid. A grease consisting of lubricating oil thickened to grease consistency with a mixture of oil soluble metal sulfonate and an alkali or alkaline earth metal acetate may be considered as an example. Salts of other low molecular weight acids, organic and inorganic, have been suggested for this purpose.

Greases of the type referred to above comprise a suitable lubricating oil, preferably mineral base lubricating oil, which may be thickened to grease consistency with about 5 to 20% by weight, based upon the total composition, of an oil soluble metal sulfonate combined with 0.5 to about 15 or 16% by weight of oil insoluble metal salt. The oil soluble metal sulfonate may be prepared in a conventional way from a sulfonic acid having a molecular weight somewhat above 400, for example 450 or 475. Such sulfonic acids are commonly obtained by treating mineral oils of suitable grade with concentrated or fuming sulfuric acid. The salts are obtained by neutralizing with metal oxide, hydroxide or carbonate.

The sulfonates of alkaline earth metals are preferred, especially strontium or calcium sulfonates, but the alkali metal sulfonates, especially sodium sulfonate, may be used for some purposes.

The oil insoluble metal salt which is mixed or complexed with the oil soluble sulfonate is preferably an alkaline earth metal salt of a low molecular weight fatty acid. Calcium acetate is a preferred material, but the corresponding salts of other low molecular weight acids, for example, the propionate, formate, butyrate, lactate, carbonate, nitrate, chloride, the sulfonates of low molecular weight such as those of methane or ethane sulfonic acids, etc., may be used. In lieu of the calcium salt, like salts of the other alkaline earth metals or of the alkali metals may be used. Mixtures of these salts can of course be employed if desired. In greases of this type, the inorganic salt attracts the oil soluble sulfonate particles to form micelles, which on a very minute scale, may be compared to tangles or "brush

2

heaps" which set up a solid structure, holding the oil in the colloid. This protective colloid is beneficial in increasing the dropping point of the grease, but when high concentrations are employed the grease is non-homogeneous. Such greases are grainy and are not satisfactory. The particles or granules in such a grease can be felt with the fingers and seen with the unaided eye. They prevent the grease from lubricating properly. They cannot be removed by filtration.

The essence of the present invention is the addition to greases of this general type of a modifier which prevents the formation of granular particles. The incorporation of the modifier, according to this invention, produces a grease which is homogeneous without being excessively soft in structure, and which retains the excellent properties such as high dropping point, resistance to bleeding, etc., of the unmodified grease.

In the preferred embodiment, the modifier is a substantially fully esterified, aliphatic polyhydric alcohol. The alcohol should have from about 2 to 10 carbon atoms, preferably 2 to 6. The esterifying groups are C<sub>12</sub> to C<sub>24</sub> fatty acid groups, the C<sub>16</sub> to C<sub>22</sub> acids being especially preferred. The trioleate ester of sorbitan is very good for this purpose. Analogous cheaper materials such as the tall oil ester of ethylene glycol or propylene glycol may be used, commercial tall oil being largely a mixture of oleic acid and abietic acid. Tall oil esters, oleate esters, and the analogous stearates, palmitates, hydroxystearates, ricinoleates, and the like, may be formed from sorbitol, sorbitan, mannitol, dulcitan, pentaerythritol, dipentaerythritol, glycerine, polyglycols, polyalkylene glycols, polyoxyalkylene glycols, and the like, with satisfactory results. Natural fats, being mixed esters of glycerol, are also suitable materials. Ordinary esters such as hydrogenated fats of natural occurrence, e. g. hydrogenated tallow may be used. The use of partial esters, such as pentaerythritol monooleate or sorbitan monooleate is possible when soft greases are desired, but when greases of firm structure are desired the completely esterified polyhydroxy alcohol is preferred.

A characteristic of these modifying materials is that when reacted with calcium acetate in the absence of sulfonate they form products varying from viscous liquids to mushy semi-solids, but in all cases the products are homogeneous. This compatibility with calcium acetate is apparently essential. Materials which are unsatisfactory for the purposes of the invention are usually not compatible with calcium acetate, for example, in hydroxy esters which precipitate a white insoluble complex and the low molecular weight esters which precipitate a granulated solid on being mixed with calcium acetate.

The preferred grease, for purposes of the present invention, comprises about 65 to 94% by weight of oil of lubricating grade, thickened with 5 to 20% of oil soluble metal sulfonates derived from the petroleum sulfonates of molecular weight above about 400. These sulfonates are combined with 0.5 to 15% of a suitable low molecular weight salt, especially the calcium salt of C<sub>1</sub> to C<sub>4</sub> aliphatic acids. This base grease material has combined with it from 0.5 to 5%, preferably from 1 to 3%, of the modifier. It is essential that the modifier be incorporated with the sulfonate prior to the addition of the calcium acetate or other oil-insoluble salt, since the addition

As indicated above, it has been found in this connection that wholly esterified polyhydric compounds are the most desirable. Hydrogenated tallow may be used and others of the most common fats and hydrogenated fats of natural origin are quite satisfactory. Partially esterified polyhydric compounds also exert a modifying action, (Examples V and VI), but they result in a grease which is much softer and not noticeably easier to handle. The following data will illustrate this point. The grease in each case was prepared as described above in Example I, except that the modifier was varied. 2% by weight of modifier was used in each case.

TABLE II  
*Effect of modifier on strontium sulfonate-calcium acetate grease*

| Ex.  | Ester                          | Type                                     | Ease of Filtering | ASTM Penetration After 10 Passes Microworker |
|------|--------------------------------|------------------------------------------|-------------------|----------------------------------------------|
| I.   | Sorbitan Trioleate             | Completely Esterified Polyhydric Alcohol | Good              | 271                                          |
| II.  | Polyoxyethylene Stearate       | do                                       | Fair              | 277                                          |
| III. | Ethylene glycol Tall Oil Ester | do                                       | Good              | 254                                          |
| IV.  | Hydrogenated Tallow            | do                                       | do                | 276                                          |
| V.   | Sorbitan Monooleate            | Partially Esterified Polyhydric Alcohol  | do                | 291                                          |
| VI.  | Ethylene glycol Monooleate     | do                                       | Fair              | 315                                          |
| VII. | Isopropyl Oleate               | Esterified Monohydric Alcohol            | Very Poor         | 260                                          |

tion of the modifier to an already formed sulfonate acetate complex is not effective.

The invention will be more fully understood by reference to the following examples:

#### EXAMPLE I

A grease prepared from 10% strontium petroleum sulfonate based on sulfonic acids of 450 molecular weight, 10% calcium acetate, and 2% sorbitan trioleate + 0.5% phenyl alpha naphthylamine dispersed in mineral base oil of 55 S. U. S. viscosity at 210° F. appears superior to a conventional soda-lime anti-friction bearing grease, showing higher dropping point (500° F. + vs. 350° F.), superior performance in the BEC bearing test at 200° F. (20% vs. 73% loss), superior wheel bearing test performance, and better oxidation stability (246 hours vs. 126 hours to 5 p. s. i. oxygen pressure drop). The apparent viscosity of the grease also is within the range generally associated with soap thickened greases as shown in attached Figure 1. By contrast, a mixture of 10% strontium sulfonate and 10% calcium acetate in the same mineral oil without the sorbitan trioleate was excessively hard and could not be filtered to a grease-like material.

The following table shows a comparison of the above grease with a conventional high grade ball bearing lubricant of substantially the same overall salt (soap) content.

TABLE I  
*Comparison with conventional bearing greases*

|                                                                             | Example I | Conventional Soda Lime Ball Bearing Lubricant |
|-----------------------------------------------------------------------------|-----------|-----------------------------------------------|
| Thickener                                                                   |           | 20-23% Sodium-Calcium Tallow Soaps.           |
| Worked Penetration, mm./10.                                                 | 274       | 299.                                          |
| Dropping Point, °F.                                                         | 500       | 350.                                          |
| BEC Test, Per Cent Loss at 210° F.                                          | 20        | 73.                                           |
| Water Wash, Per Cent Loss at 77° F.                                         | 20        | 0.                                            |
| Norma-Hoffman Test, Hours to 5 p. s. i. Drop, Wheel Bearing Test at 220° F. | 246       | 126.                                          |
|                                                                             | Pass      | Fail.                                         |

As will be obvious to those skilled in the art, various additives which are conventional in greases may be used. Materials such as antioxidants, rust inhibitors, corrosion inhibitors, extreme pressure agents, oiliness additives, and the like, may be incorporated. The type of lubricating oil may be varied widely, e. g., mineral base oil of 50 to 1000 or more S. U. S. viscosity at 100° F., or certain of the synthetic oils such as the esters of dibasic acids may be used alone or in combination with mineral oils. Conventional soap-type thickeners may be combined with the sulfonate-salt type thickeners, if desired, for example, by the incorporation of a limited amount of the soap-type thickener during grease manufacture, or by mechanical mixture of performed soap thickened grease with the sulfonate-type grease.

In the appended claims, "mineral base" oil refers to oils which are essentially or predominantly of petroleum derivation, but may also include significant amounts of conventional synthetics, thickeners, and the like, as will be obvious to those skilled in the art.

What is claimed is:

1. A lubricating grease composition consisting essentially of a lubricating oil thickened to a grease consistency with a complex combined thickener of 5 to 20% by weight, based on the total composition, of oil soluble metal sulfonate derived from relatively high molecular weight petroleum sulfonic acids combined with 0.5 to 15% by weight of an oil insoluble metal salt of relatively low molecular weight acid, and a structure modifier comprising 0.1 to 5% of an ester of polyhydric alcohol and organic acid of 12 to 24 carbon atoms.

2. Composition of claim 1 wherein said structure modifier is a C<sub>12</sub> to C<sub>24</sub> fatty acid substantially complete ester of an aliphatic polyhydric alcohol.

3. Composition of claim 1 wherein said structure modifier is a substantially complete C<sub>12</sub> to C<sub>24</sub> fatty acid ester of an aliphatic polyhydric alcohol of 2 to 6 hydroxyl groups.

4. Composition of claim 1 wherein said structure modified is a substantially complete C<sub>18</sub> fatty acid ester of an aliphatic polyhydric alcohol.

5. Composition of claim 1 wherein said structure modifier is a substantially complete C<sub>18</sub> ester of sorbitan.

6. Composition of claim 1 wherein said structure modifier is hydrogenated tallow.

7. Composition as in claim 1 in which said structure modifier is polyoxyethylene stearate.

8. Composition of claim 1 in which said structure modifier is a substantially complete ester of a partially dehydrated hexahydric alcohol.

9. A lubricating grease composition consisting essentially of 65 to 94% by weight of mineral base lubricating oil, 5 to 20% based on the total composition of oil a complex combined thickener comprising soluble metal sulfonate derived from petroleum base sulfonic acids of at least 400 molecular weight, 0.5 to 15% of alkaline earth metal salt of C<sub>1</sub> to C<sub>4</sub> fatty acid, and 0.1 to 5% of a substantially fully esterified C<sub>12</sub> to C<sub>24</sub> fatty acid ester of a partially dehydrated polyhydric alcohol.

10. Composition as in claim 9 wherein said ester is a C<sub>16</sub> to C<sub>20</sub> tri-ester of sorbitan.

11. Composition as in claim 9 wherein said ester is sorbitan esterified with at least two oleate groups.

12. Composition as in claim 9 wherein said ester is sorbitan trioleate.

13. Composition as in claim 9 wherein said ester is ethylene glycol tall oil ester.

14. A lubricating grease composition consisting essentially of lubricating oil, thickened to a

grease consistency with a complex thickener comprising a mixture of oil soluble strontium petroleum sulfonate and calcium acetate, and from 0.1 to 5% by weight, based on the total composition, of a substantially fully esterified C<sub>16</sub> to C<sub>20</sub> fatty acid ester of an aliphatic polyhydric alcohol which has 2 to 6 carbon atoms.

15. A method for preparing a lubricating grease which comprises blending about 65-94% by weight based on the total composition of a mineral base lubricating oil, 5 to 20% of an oil soluble metal sulfonate derived from petroleum base sulfonic acids and 0.1 to 5% of an ester of polyhydric alcohol and organic acid of 12 to 24 carbon atoms, forming a homogeneous mixture of the aforesaid ingredients, and thereafter incorporating 0.5 to 15% by weight of an oil insoluble metal salt of a relatively low molecular weight acid to form with said sulfonate a complex thickener.

ROSEMARY O'HALLORAN.

#### REFERENCES CITED

The following references are of record in the file of this patent:

#### UNITED STATES PATENTS

| Number     | Name             | Date          |
|------------|------------------|---------------|
| 2,070,781  | Brunstrum et al. | Feb. 16, 1937 |
| 2,303,558  | Kaugman et al.   | Dec. 1, 1942  |
| 2,398,173  | Brunstrum et al. | Apr. 9, 1946  |
| 2,399,063  | Schantz          | Apr. 23, 1946 |
| 2,417,429  | McLennan         | Mar. 18, 1947 |
| 2,468,098  | Morway et al.    | Apr. 26, 1949 |
| 2,475,589  | Bondi            | July 12, 1949 |
| Re. 23,082 | Zimmer et al.    | Jan. 25, 1949 |